

2,703,784

CORROSION INHIBITORS AND COMPOSITIONS  
CONTAINING THE SAMEEllis K. Fields, Chicago, Ill., assignor to Standard Oil  
Company, Chicago, Ill., a corporation of IndianaNo Drawing. Application October 31, 1952,  
Serial No. 318,091

37 Claims. (Cl. 252—32.7)

This invention relates to new compositions of matter which are effective corrosion inhibitors and which are non-corrosive to silver, silver alloys and similar metal. More particularly, the invention pertains to lubricant compositions containing the new compositions of matter which are non-corrosive to such metals and inhibit the corrosion thereof by sulfur and/or corrosive sulfur-containing compounds.

Advances in the design and construction of internal combustion engines to produce improved and more efficient and economical engines have presented many problems in the lubrication of the modern internal combustion engine. To meet the increased severe demands upon engine lubricants, many types of lubricant additives have been developed to obtain certain desired characteristics thereof. Among the more effective addition agents which have been developed for compounding with lubricants are many sulfur-containing organic compounds, such as by way of example, sulfurized terpenes, sulfurized hydrocarbon oils, vegetable oils or animal oils, xanthate esters, organic polysulfides, particularly polyalkyl polysulfides, metal salts of organo-substituted thioacids of phosphorus, metal salts of the reaction product of a phosphorus sulfide and a hydrocarbon, such as for example, polybutenes and other polyolefins, and combinations of the foregoing.

Recent increased use of silver and similar metal in the construction of improved internal combustion engines has created new problems in the use of sulfur-containing additives in lubricants for such engines; the primary problem created being the corrosion of such silver parts of the engine by the sulfur-containing additives. While such corrosion can be eliminated by avoiding the use of sulfur-containing additives in lubricants for such engines, this solution of the problem is accompanied by the loss of the highly desired beneficial effects of the additives of this type.

It is an object of the present invention to provide a non-corrosive composition of matter. Another object of the invention is to provide a composition non-corrosive to silver and similar metal. A still further object of the invention is to provide a composition which will inhibit the corrosion of silver and similar metal by sulfur and/or organo sulfur-containing compounds. A still further object of the invention is to provide a lubricant composition which is non-corrosive. Still another object of the invention is to provide a lubricant composition containing an addition agent which will inhibit the corrosion of silver and similar metal by sulfur and/or organo sulfur-containing compounds. A further object of the invention is to provide a method of inhibiting the corrosion of silver and similar metal. Still another object of the invention is to provide a method of lubricating internal combustion engines containing silver and similar metal parts and inhibiting the corrosion of such metals by lubricants which contain sulfur and/or organo sulfur-containing compounds.

In accordance with the present invention, the new composition of matter is the oil-soluble reaction product of an aldehyde, a mercaptan and 2,5-dimercapto-1,3,4-thiadiazole in the molar ratio of from about 2:2:1 to 10:2:9, and preferably in the molar ratio of 2:2:1. In general, the reaction is carried out by adding an aldehyde to a mixture of the mercaptan and the dimercapto-thiadiazole, and heating the mixture at temperatures of from about 40° C. to about 140° C. for a period of from twenty minutes to about sixteen hours. Preferably, the reaction is carried out in the presence of a suitable solvent, such

as by way of example, dioxane, ethylene glycol, di-methyl and di-ethyl ethers, and diethylene glycol di-methyl and di-ethyl ethers. At the end of the reaction period, the solvent and the water, produced in the reaction, are removed from the reaction product, preferably by stripping in a vacuum, and the stripped product filtered, if necessary.

The aldehyde employed may be an aliphatic, an aromatic, or a heterocyclic aldehyde of from about 1 to about 20 or more carbon atoms, and may contain substituents, such as alkoxy, hydroxy, alkyl mercapto, halogen or nitro groups. Examples of suitable aldehydes are formaldehyde, acetaldehyde, benzaldehyde, 2-ethylhexyl aldehyde, butyraldehyde, heptaldehyde, caprylic aldehyde, acrylic aldehyde, crotonaldehyde, vinyl acetaldehyde, phenyl acetaldehyde, nitrobenzaldehyde, salicyaldehyde, furfural, chloral, etc. Any mercaptan can be employed in the reaction although an aliphatic or aromatic mono- or poly-mercaptan containing from about 1 to about 30 carbon atoms, and preferably from about 6 to about 20 carbon atoms, is preferred. Examples of suitable mercaptans are ethyl mercaptan, butyl mercaptan, hexyl mercaptan, octyl mercaptan, nonyl mercaptan, octadecyl mercaptan, thiophenol, etc.

The preparation of the above-described reaction products is illustrated by the following examples, which are given by way of illustration and are not intended to limit the scope of the invention.

## EXAMPLE I

30 A mixture of 60 grams (0.4 mol.) of 2,5-dimercapto-1,3,4-thiadiazole and 116.8 grams (0.8 mol.) tertiary octyl mercaptan was dissolved in 300 cc. dioxane at 70° C. To the stirred hot solution was added, drop-wise, 66 cc. of 36% aqueous formaldehyde over a thirty minute period. Stirring was continued at 100° C. for one and one-half hours and the mixture then stripped in vacuo and filtered through celite. A yield of 143 grams of a viscous yellow product was obtained which analyzed as follows:

|          | Per cent |
|----------|----------|
| Carbon   | 44.22    |
| Hydrogen | 6.35     |
| Sulfur   | 37.0     |
| Nitrogen | 7.9      |

## EXAMPLE II

50 To a solution of 45 grams (0.3 mol.) of 2,5-dimercapto-1,3,4-thiadiazole and 121.2 grams (0.6 mol.) of tertiary dodecyl mercaptan in 200 cc. dioxane, heated to 65° C., was added, drop-wise, 49.5 cc. 36% aqueous formaldehyde over a twenty minute period. The mixture was stirred for two and one-half hours at 100° C., stripped in vacuo and filtered through celite. A yield of 154 grams of a viscous yellow product was obtained which analyzed as follows:

|          | Per cent |
|----------|----------|
| Carbon   | 56.16    |
| Hydrogen | 8.76     |
| Sulfur   | 26.9     |
| Nitrogen | 4.63     |

## EXAMPLE II

65 A mixture of 30 grams (.2 mol.) 2,5-dimercapto-1,3,4-thiadiazole, 58.4 grams (0.4 mol.) tertiary octyl mercaptan and 51.2 grams (0.4 mol.) 2-ethylhexaldehyde in 75 cc. dioxane, was heated at 115° C. for four hours, stripped in vacuo to remove the diluent and the water of reaction, and filtered through celite. 100 grams of a viscous yellow product was obtained.

## EXAMPLE IV

70 A mixture of 45 g. (.3 mole) 2,5-dimercapto-1,3,4-thiadiazole and 102 cc. (.6 mole) t-octyl mercaptan was stirred at 90° C. and treated drop-wise with 61 cc. benzaldehyde over a 35 minute period. The mixture was stirred at 100° C. for 2 hours, stripped in vacuo and filtered through celite plus a little alumina. The product, 175 g., was a very viscous yellow-orange liquid completely soluble in naphtha. The product contained 27.4% sulfur and 4.9% nitrogen.

3  
EXAMPLE V

50 cc. of furfural (.6 mole) was added, drop-wise, to a mixture of 102 cc. (.6 mole) t-octyl mercaptan and 45 grams (.3 mole) 2,5-dimercapto-1,3,4-thiadiazole and the mixture stirred for two hours at a temperature of 90° C. The reaction product was then stripped in vacuo and filtered while warm. The product, 120 grams, was a dark purple viscous material having a sulfur content of 25.1% and a nitrogen content of 4.4%.

## EXAMPLE VI

To a stirred mixture of 41 cc. (.4 mole) thiophenol and 30 g. (.2 mole) 2,5-dimercapto-1,3,4-thiadiazole at 75-80° C. was added 56 cc. (0.4 mole) heptaldehyde, drop-wise, over a 15 minute period. Stirring was continued for two hours at 100° C. The mixture was stripped at 120° C., and 4 millimeters pressure, then filtered hot through a little celite. The product, 94 g., was a viscous-orange oil.

Instead of reacting 2,5-dimercapto-1,3,4-thiadiazole with the mercaptan and aldehyde as above described in the preparation of the additive, we may carry out the reaction by forming in situ the dimercapto-thiadiazole and reacting the same with the aldehyde and mercaptan as illustrated by the following example:

## EXAMPLE VII

To a mixture of 150 grams of cracked ice and 130.5 cc. of 84% hydrazine hydrate was added 280 cc. of carbon disulfide over a period of 10 minutes. While cooling the mixture externally, a solution of 180 grams of sodium hydroxide in 325 cc. of water and 30 cc. of ethyl alcohol was added drop-wise to the cooled mixture while maintaining a temperature of about 50° C. or lower. The mixture was then stirred and refluxed at 85° C. for three hours, cooled and acidified with 120 cc. of concentrated sulfuric acid diluted with 200 grams of ice. To the resulting slurry of 2,5-dimercapto-1,3,4-thiadiazole in sodium sulfate solution was added 1000 cc. of tertiary octyl mercaptan, and then with vigorous agitation was added, drop-wise, 374 cc. of 37% aqueous formaldehyde. The resultant mixture was heated at 85° C. for two hours and cooled to room temperature (about 23° C.). The mixture separated into a lower solidified layer of sodium sulfate and an upper liquid layer. The latter was decanted, treated with 10 grams of sodium bicarbonate, then stripped in vacuo, and filtered through celite; 610 grams of a light yellow liquid product was obtained.

The above-described reaction products are effective corrosion inhibitors, particularly with respect to silver and similar metals when used in combination with lubricant base oils, such as hydrocarbon oils, synthetic hydrocarbon oils, such as those obtained by the polymerization of hydrocarbons, such as olefin polymers, for example, polybutenes, polypropylene and mixtures thereof, etc.; synthetic lubricating oils of the alkylene-oxide type, for example, the "Ucon oils," marketed by Carbide and Carbon Corporation, as well as other synthetic oils, such as the polycarboxylic acid ester type oils, such as the esters of adipic acid, sebatic acid, maleic acid, azelaic acid, etc. The herein-described reaction products are effectively used in such lubricants in concentrations of from about 0.02% to about 10%, and preferably from about 0.05% to about 5%.

While the above-described reaction products can be suitably employed alone in combination with a base oil, they are usually used in combination with other lubricant addition agents, which impart various desired characteristics to the base oil. Usually, these reaction products are used in conjunction with detergent-type additives, particularly those which contain sulfur or phosphorus and sulfur. The additives of this type are usually used in amounts of from about 0.002% to about 10%, and preferably from about 0.01% to about 5%. Among the phosphorus and sulfur-containing addition agents are the neutralized reaction products of a phosphorus sulfide, and a hydrocarbon, an alcohol and a ketone, an amine or an ester. Of the phosphorus sulfide reaction product additives, we prefer to employ the neutralized reaction products of a phosphorus sulfide, such as phosphorus pentasulfide, and a hydrocarbon of the type described in U. S. 2,316,082 issued to C. M. Loane et al., April 6, 1943. As taught in this patent, the preferred hydrocarbon constituent of the reaction is a mono-olefin hydrocarbon polymer resulting from the polymerization of low molecular weight mono-olefin hydrocarbons, such as propyl-

enes, butenes, amylenes or copolymers thereof. Such polymers may be obtained by the polymerization of mono-olefins of less than 6 carbon atoms in the presence of a catalyst, such as sulfuric acid, phosphoric acid, boron fluoride, aluminum chloride, or other similar halide catalysts of the Friedel-Crafts type.

The polymers employed are preferably mono-olefin polymers or mixtures of mono-olefin polymers and iso-mono-olefin polymers having molecular weights ranging from about 150 to about 50,000, or more, and preferably from about 500 to about 10,000. Such polymers can be obtained, for example, by the polymerization in the liquid phase of a hydrocarbon mixture containing mono-olefins and isomono-olefins, such as butylene and isobutylene at a temperature of from about -80° F. to about 100° F. in the presence of a metal halide catalyst of the Friedel-Crafts type, such as for example, boron fluoride, aluminum chloride, and the like. In the preparation of these polymers, a hydrocarbon mixture containing isobutylene, butylenes and butanes recovered from petroleum gases especially those gases produced in the cracking of petroleum oils in the manufacture of gasoline can be used.

Another suitable polymer is that obtained by polymerizing in the liquid phase a hydrocarbon mixture comprising substantially C<sub>3</sub> hydrocarbons in the presence of an aluminum chloride-complex catalyst. The catalyst is preferably prepared by heating aluminum chloride with isooctane. The hydrocarbon mixture is introduced into the bottom of the reactor and passed upwardly through the catalyst layer, while a temperature of from about 50° F. to about 110° F. is maintained in the reactor. The propane and other saturated gases pass through the catalyst while the propylene is polymerized under these conditions. The propylene polymer can be fractionated to any desired molecular weight, preferably from about 500 to about 1000 or higher.

Other suitable polymers are those obtained by polymerizing a hydrocarbon mixture containing about 10% to about 25% isobutylene at a temperature of from about 0° F. to about 100° F., and preferably 0° F. to about 32° F. in the presence of boron fluoride. After the polymerization of the isobutylene together with a relatively minor amount of the normal olefins present, the reaction mass is neutralized, washed free of acidic substances and the unreacted hydrocarbons subsequently separated from the polymers by distillation. The polymer mixture so obtained, depending upon the temperature of reaction, varies in consistency from a light liquid to viscous oily material and contains polymers having molecular weights ranging from about 100 to about 2000, or higher. The polymers so obtained may be used as such, or the polymer may be fractionated under reduced pressure into fractions of increasing molecular weights and suitable fractions obtained reacted with the phosphorus sulfide to obtain the desired reaction products. The bottoms resulting from the fractionation of the polymer which may have Saybolt Universal viscosities at 210° F. ranging from about 50 seconds to about 10,000 seconds, are well suited for this purpose.

Essentially paraffinic hydrocarbons, such as bright stock residuums, lubricating oil distillates, petrolatums or paraffin waxes may be used. There can also be employed the condensation products of any of the foregoing hydrocarbons, usually through first halogenating the hydrocarbons with aromatic hydrocarbons in the presence of anhydrous inorganic halides, such as aluminum chloride, zinc chloride, boron fluoride, and the like.

Examples of other high molecular weight olefinic hydrocarbons, which can be employed, are cetene (C<sub>16</sub>), cerotene (C<sub>28</sub>), meline (C<sub>30</sub>), and mixed high molecular weight alkenes obtained by cracking petroleum oils.

Other preferred olefins suitable for the preparation of the phosphorus sulfide reaction products are olefins having at least 20 carbon atoms in the molecule of which from about 13 carbon atoms to about 18 carbon atoms, and preferably at least 15 carbon atoms are in a long chain. Such olefins can be obtained by the dehydrogenation of paraffins, such as by cracking of paraffin waxes or by the dehalogenation of alkyl halides, preferably long chain alkyl halides, particularly halogenated paraffin waxes.

As a starting material there can be used the polymer or synthetic lubricating oil obtained by polymerizing unsaturated hydrocarbons resulting from the vapor phase cracking of paraffin waxes in the presence of aluminum

chloride which is fully described in United States Patents Nos. 1,955,260, 1,970,402 and 2,091,398. Still another type of olefin polymer which may be employed is the polymer resulting from the treatment of vapor phase cracked gasoline and/or gasoline fractions with sulfuric acid or solid adsorbents, such as fuller's earth, whereby unsaturated polymerized hydrocarbons are removed. The reaction products of the phosphorus sulfide and the polymers resulting from the volatilization of hydrocarbons as described, for example, in United States Patents Nos. 2,197,768 and 2,191,787 are also suitable.

Other hydrocarbons that can be reacted with a phosphorus sulfide are aromatic hydrocarbons, such as for example, benzene, naphthalene, toluene, xylene, diphenyl, and the like, or with an alkylated aromatic hydrocarbon, such as for example, benzene having an alkyl substituent having at least four carbon atoms, and preferably at least eight carbon atoms, such as a long chain paraffin wax.

The phosphorus sulfide-hydrocarbon reaction product can be readily obtained by reacting a phosphorus sulfide, for example,  $P_2S_5$  with the hydrocarbon at a temperature of from about 200° F. to about 500° F., and preferably from about 200° F. to about 400° F., using from about 1% to about 50%, and preferably from about 5% to about 25% of the phosphorus sulfide in the reaction. It is advantageous to maintain a non-oxidizing atmosphere, such as for example, an atmosphere of nitrogen above the reaction mixture. Usually, it is preferable to use an amount of the phosphorus sulfide that will completely react with the hydrocarbon so that no further purification becomes necessary; however, an excess amount of phosphorus sulfide can be used and separated from the product by filtration or by dilution with a hydrocarbon solvent, such as hexane, filtering and subsequently removing the solvent by suitable means, such as by distillation. If desired, the reaction product can be further treated with steam at an elevated temperature of from about 100° F. to about 600° F.

The phosphorus sulfide-hydrocarbon reaction product normally shows a titratable acidity which is neutralized by treatment with a basic reagent. The phosphorus sulfide-hydrocarbon reaction product, when neutralized with a basic reagent, containing a metal constituent, is characterized by the presence or retention of the metal constituent of the basic reagent.

The neutralized phosphorus sulfide-hydrocarbon reaction product can be obtained by treating the acidic reaction product with a suitable basic compound, such as hydroxide, carbonate, oxide or sulfide of an alkaline earth metal or an alkali metal, such as for example, potassium hydroxide, sodium hydroxide, sodium sulfide, calcium oxide, lime, barium hydroxide, barium oxide, etc. Other basic reagents can be used, such as for example, ammonia or an alkyl or aryl-substituted ammonia, such as amines. The neutralization of the phosphorus sulfide-hydrocarbon reaction product is carried out preferably in a non-oxidizing atmosphere by contacting the acidic reaction product either as such or dissolved in a suitable solvent, such as naphtha with a solution of the basic agent. As an alternative method, the reaction product can be treated with solid alkaline compounds, such as KOH, NaOH,  $Na_2CO_3$ ,  $K_2CO_3$ , CaO, BaO,  $Ba(OH)_2$ ,  $Na_2S$ , and the like, at an elevated temperature of from about 100° F. to about 600° F. Neutralized reaction products containing a heavy metal constituent such as for example, tin, titanium, aluminum, chromium, cobalt, zinc, iron, and the like, can be obtained by reacting a salt of the desired heavy metal with the phosphorus sulfide-hydrocarbon reaction product which has been treated with the phosphorus sulfide-hydrocarbon reaction product, which has been treated with a basic reagent, such as above described.

Other phosphorus sulfide-reaction products which can be used are the reaction products of a phosphorus sulfide and a fatty acid ester of the type described in U. S. 2,399,243; the phosphorus sulfide-degras reaction products of U. S. 2,413,332; the reaction product of an alkylated phenol with the condensation product of  $P_2S_5$  and turpentine of U. S. 2,409,877 and U. S. 2,409,878; the reaction product of a phosphorus sulfide and stearonitrile of U. S. 2,416,807; etc.

The silver corrosion inhibiting property of the above-described dimercapto-thiadiazole reaction products is demonstrated by the data in Table I, which were obtained

by subjecting mixtures of hydrocarbon oil, a neutralized reaction product of  $P_2S_5$  and a polybutene, and various 2,5-dimercapto-1,3,4-thiadiazole reaction products to the following test, hereinafter referred to as the modified E. M. D. test:

A silver strip 2 cm. x 5.5 cm. with a small hole at one end for suspension, is lightly abraided with No. 0 steel wool, wiped free of any adhering steel wool, washed with carbon tetrachloride, air-dried and then weighed to 0.1 milligram. 300 cc. of the oil to be tested is placed in a 500 cc. lipless glass beaker and the oil heated to a temperature of 300° F. ( $\pm 2^\circ$  F.) and the silver test strip suspended in the oil so that the strip is completely immersed therein. The oil in the beaker is stirred by means of a glass stirrer operating at 300 R. P. M. At the end of twenty-four hours, the silver strip is removed, and while still hot, rinsed thoroughly with carbon tetrachloride and air-dried. The appearance of the strip is then visually noted and given ratings according to the following scale:

- 1—Bright
- 2—Stained
- 3—Grey-black
- 4—Black, smooth
- 5—Black, flake

After the visual inspection, the silver strip is immersed in an 10% potassium cyanide solution at room temperature until the silver surface assumes its original bright or silver appearance. The silver strip is then washed successively with distilled water and acetone, air-dried and weighed.

The following lubricant compositions were subjected to the above test and the results obtained tabulated in Table I.

35 *Sample A.*—Control (solvent extracted SAE 30 oil + 3.3% barium-containing neutralized reaction product of  $P_2S_5$  and a polybutene of about 1000 molecular weight).

*Sample B.*—A + 0.75% reaction product of Example I.

*Sample C.*—A + 0.75% reaction product of Example II.

*Sample D.*—A + 0.75% reaction product of Example III.

*Sample E.*—A + 0.75% reaction product of Example IV.

*Sample F.*—A + 0.75% reaction product of Example V.

*Sample G.*—A + 0.75% reaction product of Example VII.

Table I

| Sample | Silver Corrosion (Wt. Loss, Mg.) |
|--------|----------------------------------|
| A      | 20-25                            |
| B      | 0/1                              |
| C      | 0/1                              |
| D      | 0/1                              |
| E      | 0/1                              |
| F      | 0/1                              |
| G      | 0/1                              |

Since a weight loss of 20 milligrams is allowable, the ability of the 2,5-dimercapto-1,3,4-thiadiazole derivatives of this invention to inhibit silver corrosion is demonstrated by the above data.

The effectiveness of the herein-described dimercapto-thiadiazole reaction products in inhibiting corrosion of copper and/or lead-containing metals, such as for example, copper-lead alloys, is demonstrated by the data in Table II, obtained by subjecting lubricants containing the additive to the following test:

A copper-lead test specimen is lightly abraided with steel wool, washed with naphtha, dried and weighed to the nearest milligram. The cleaned copper-lead test specimen is suspended in a steel beaker, cleaned with a hot trisodium phosphate solution, rinsed with water, acetone and dried, and 250 grams of the oil to be tested, together with 0.625 gram lead oxide and 50 grams of a 30-35 mesh sand charged to the beaker. The beaker is then placed in a bath or heating block and heated to a temperature of 300° ( $\pm 2^\circ$  F.), while the contents are stirred by means of a stirrer rotating at 750 R. P. M. The contents of the beaker are maintained at this temperature for twenty-four hours, after which the copper-lead test specimen is removed, rinsed with naphtha, dried

Table III

| Sample | 1 |
|--------|---|
| A'     |   |
| B'     |   |
| C'     |   |
| D'     |   |
| E'     |   |
| F'     |   |
| G'     |   |
| H'     |   |

and weighed. The test specimen is then replaced in the beaker and an additional 0.375 grams of lead oxide added to the test oil. At the end of an additional twenty-four hours of test operation, the test specimen is again removed, rinsed and dried as before, and weighed. The test specimen is again placed in the beaker together with an additional 0.250 grams of lead oxide and the test continued for another twenty-four hours (seventy-two hours total). At the conclusion of this time, the test specimen is removed from the beaker, rinsed in naphtha, dried and weighed.

The loss in weight of the test specimen is recorded after each weighing.

This test, known as the Sand Stirring Corrosion Test, is referred to hereinafter as "SSCT."

The data obtained when subjecting lubricant compositions, designated Samples A to E and G, above, to the foregoing test, are tabulated in Table II.

Table II

| Sample   | S. S. C. T., Mg. Wt. Loss |         |         |
|----------|---------------------------|---------|---------|
|          | 24 Hrs.                   | 48 Hrs. | 72 Hrs. |
| Sample A | 305                       | 580     | 850     |
| Sample B | 19                        | 29      | 42      |
| Sample C | 21                        | 108     | 298     |
| Sample D | 9                         | 11      | 64      |
| Sample E | 16                        | 18      | 371     |
| Sample G | 0                         | 3       | 46      |

Since weight losses of 200 milligrams in 48 hours and 500 milligrams in 72 hours are allowable, the corrosion inhibiting property of the herein-described 2,5-dimercapto-1,3,4-thiadiazole derivatives is clearly demonstrated by the above data.

Under certain conditions, it is desirable to use in lubricant compositions from about 0.01% to about 5%, and preferably from about 0.1% to about 2%, elemental sulfur or an organic sulfur-containing compound of the type hereinabove described, either alone or in combination with other additives. Effective lubricant compositions are obtained by the combination of the neutralized reaction products of a phosphorus sulfide and a hydrocarbon, as above described, with elemental sulfur or an organic sulfur-containing compound, such as sulfurized mineral oils, sulfurized non-drying animal and vegetable oils, sulfurized olefins and olefin polymers, sulfurized sperm oil, etc., as described and claimed in U. S. Reissue No. 22,464 issued to C. D. Kelso et al. April 4, 1944, or with sulfurized terpenes, for example, dipentene as described and claimed in U. S. 2,422,583 issued to T. H. Rogers et al. June 17, 1947. While these compounds impart highly desired characteristics to lubricants, and effectively inhibit the corrosion of copper and/or lead, they are corrosive to silver and similar metals, and for this reason, lubricants containing such addition agents fail to pass the above-described E.M.D. test. In accordance with the present invention, however, the incorporation in such lubricant compositions of small amounts, namely from about 0.1% to about 10%, and preferably from about 0.25% to about 5% of the herein-described 2,5-dimercapto-1,3,4-thiadiazole reaction products, effectively inhibits the corrosiveness of the silver corrosive compounds without impairing their other desired properties.

The ability of the herein-described 2,5-dimercapto-1,3,4-thiadiazole derivatives to inhibit the silver corrosion tendency of active sulfur-containing organic compounds is demonstrated by the following E. M. D. data in Table III, obtained with the following compositions:

Sample A'—(Control).—Solvent extracted SAE-30 mineral oil + 3.3% barium-containing neutralized reaction product of  $\text{PbS}_2$  and a polybutene of about 1000 molecular weight + 0.75% sulfurized dipentene.

Sample B'—A' + 0.10% product of Example I, supra.

Sample C'—A' + 0.15% product of Example I, supra.

Sample D'—A' + 0.15% product of Example II, supra.

Sample E'—A' + 0.15% product of Example III, supra.

Sample F'—A' + 0.15% product of Example IV, supra.

Sample G'—A' + 0.15% product of Example V, supra.

Sample H'—A' + 0.15% product of Example VII, supra.

As indicated by the above data, the herein-described 2,5-dimercapto-1,3,4-thiadiazole derivatives exhibit corrosion tendencies of active sulfur-containing organic compounds, i. e., sulfurized terpenes toward lead. However, these derivatives do not deleteriously affect the corrosion inhibiting properties of the sulfur-containing organic compounds towards metals, such as copper.

Although the invention has been described in connection with the use of the herein-described 2,5-dimercapto-1,3,4-thiadiazole derivatives in combination with more secondary additives in lubricant compositions, the invention is not restricted to such use since these additives find utility when used alone in various lubricant positions or hydrocarbon oil compositions to improve and desired characteristics thereto. Thus, for example, these derivatives may be used alone in lubricating oils to impart desired properties thereto, such as in the oxidation of hydrocarbon oils as demonstrated in Table IV. These data were obtained by adding hydrocarbon oils containing various above-described derivatives to the following oxidation test herein referred to as the I. S. O. T. In this test 250 cc. of the oil to be tested are heated at 330° F. to 332° F. in a glass beaker in the presence of 5 square millimeters of copper and 10 square millimeters of iron. Four rods of 6 mill. diameter are suspended in the oil and stirred at about 1300 R. P. M. by means of a stirrer. At intervals of twenty-four, forty-eight, seventy-two hours, oil samples are taken and the acidity and viscosity values determined. The following oil compositions were subjected to the above test, and the results tabulated in Table IV.

Sample A''—(Control).—Solvent extracted SAE-30 mineral oil.

Sample B''—A'' + 0.5% of the product of Example I, supra.

Sample C''—A'' + 1.0% of the product of Example I, supra.

Table IV

| Sample | Acidity (Mg. KOH/gr. Oil) |         |         | Naphtha, Insoluble |         |         |
|--------|---------------------------|---------|---------|--------------------|---------|---------|
|        | 24 hrs.                   | 48 hrs. | 72 hrs. | 24 hrs.            | 48 hrs. | 72 hrs. |
| A''    | 3.36                      | 6.72    | 9.8     | 0.120              | 5.00    | 6.71    |
| B''    | 1.4                       | 3.08    | 9.8     | 0.071              | 1.143   | 4.86    |
| C''    | 1.68                      | 2.52    | 5.88    | 0.043              | 1.28    | 4.00    |

In addition to the aforementioned detergent-type additives and corrosion inhibitors, compositions containing the herein-described derivatives of 2,5-dimercapto-1,3,4-thiadiazoles can contain other additives, such as antioxidants, pourpoint depressors, extreme pressure agents, wear agents, V. I. improvers, etc.

While this invention has been described in connection with the use of the herein-described additives and lubricant compositions, their use is not limited thereto but can be used in products other than lubricating oils, such as for example, fuel oils, insulating oils, greases, drying animal and vegetable oils, waxes, asphalts and for internal combustion engines, particularly where the corrosion must be inhibited.

Unless otherwise stated, percentages given herein in the appended claims are weight percentages.

Soluble oil compositions containing the herein-described derivatives of 2,5-dimercapto-1,3,4-thiadiazoles are claimed and claimed reaction products of an aldehyde, a melanin, and 2,5-dimercapto-1,3,4-thiadiazole are claimed copending Roberts et al. application Serial No. 339 filed February 27, 1953.

Although the present invention has been described in reference to specific preferred embodiments thereof,

invention is not to be considered as limited thereto, but includes within its scope such modifications and variations as come within the spirit of the appended claims.

I claim:

1. A new composition of matter, the reaction product of an aldehyde, a mercaptan selected from the class consisting of an aliphatic mercaptan and an aromatic mercaptan and 2,5-dimercapto-1,3,4-thiadiazole, said reaction product having corrosion inhibiting properties and being suitable for addition to oils to impart corrosion inhibiting characteristics thereto, said aldehyde, mercaptan and 2,5-dimercapto-1,3,4-thiadiazole being reacted in the molar ratio of from about 2:2:1, respectively, to about 10:2:9, respectively.

2. A composition of matter as described in claim 1 in which the aldehyde is an aliphatic aldehyde of from 1 to about 20 carbon atoms.

3. A composition of matter as described in claim 2 in which the aliphatic aldehyde is formaldehyde.

4. A composition of matter as described in claim 2 in which the aliphatic aldehyde is 2-ethyl hexaldehyde.

5. A new composition of matter as described in claim 1 in which the aldehyde is an aromatic aldehyde.

6. A new composition of matter as described in claim 5 in which the aromatic aldehyde is benzaldehyde.

7. A new composition of matter as described in claim 5 in which the aromatic aldehyde is salicyaldehyde.

8. A new composition of matter as described in claim 1 in which the aldehyde is a heterocyclic aldehyde.

9. A new composition of matter as described in claim 8 in which the heterocyclic aldehyde is furfural.

10. A new composition of matter as described in claim 1 in which the mercaptan is octyl mercaptan.

11. A new composition of matter as described in claim 1 in which the mercaptan is dodecyl mercaptan.

12. A new composition of matter as described in claim 1 in which the mercaptan is thiophenol.

13. A composition comprising a major proportion of an oleaginous compound and from about 0.02% to about 10% of a reaction product of an aldehyde, a mercaptan selected from the class consisting of an aliphatic mercaptan and an aromatic mercaptan, and 2,5-dimercapto-1,3,4-thiadiazole, said aldehyde, mercaptan and 2,5-dimercapto-1,3,4-thiadiazole being reacted in the molar ratio of from about 2:2:1, respectively, to about 10:2:9, respectively.

14. A composition as described in claim 13 in which the aldehyde is an aliphatic aldehyde of from 1 to about 20 carbon atoms.

15. A composition as described in claim 14 in which the aldehyde is formaldehyde.

16. A composition as described in claim 14 in which the aldehyde is 2-ethyl hexaldehyde.

17. A composition as described in claim 13 in which the aldehyde is an aromatic aldehyde.

18. A composition as described in claim 17 in which the aromatic aldehyde is benzaldehyde.

19. A composition as described in claim 13 in which the aldehyde is a heterocyclic aldehyde.

20. A composition as described in claim 19 in which the aldehyde is furfural.

21. A composition as described in claim 13 in which the mercaptan is octyl mercaptan.

22. A composition as described in claim 13 in which the mercaptan is dodecyl mercaptan.

23. A composition as described in claim 13 in which the mercaptan is thiophenol.

24. A composition comprising a major proportion of an oleaginous compound, from about 0.02% to about 10% of the reaction product of an aldehyde, an aliphatic mercaptan having from 1 to about 30 carbon atoms, and 2,5-dimercapto-1,3,4-thiadiazole in the molar ratio of from about 2:2:1 respectively to 10:2:9 respectively, and from about 0.001% to about 10% of a sulfur-containing organic compound normally corrosive to silver.

25. A composition as described in claim 24 in which the sulfur-containing organic compound is a sulfurized terpene.

26. A lubricant composition comprising a major propor-

tion of an oleaginous compound, from about 0.02% to about 10% of the reaction product of an aldehyde, an aliphatic mercaptan and from about 1 to about 30 carbon atoms, and 2,5-dimercapto-1,3,4-thiadiazole in the molar ratio of from about 2:2:1 to 10:2:9 and from about 0.001% to about 10% of a phosphorus and sulfur-containing detergent-type lubricant additive.

27. A lubricant composition as described in claim 26 in which the phosphorus and sulfur-containing detergent-type lubricant additive is a neutralized reaction product of a phosphorus sulfide and a hydrocarbon.

28. A lubricant composition as described in claim 26 in which the phosphorus and sulfur-containing detergent-type lubricant additive is an alkali metal-containing neutralized reaction product of a phosphorus sulfide and an olefin polymer.

29. A lubricant composition as described in claim 26 in which the phosphorus and sulfur-containing lubricant additive is a potassium-containing neutralized reaction product of a phosphorus sulfide and an olefin polymer.

30. A lubricant composition as described in claim 26 in which the phosphorus and sulfur-containing detergent-type lubricant additive is an alkaline-earth-containing neutralized reaction product of a phosphorus sulfide and an olefin polymer.

31. A lubricant composition described in claim 26 in which the phosphorus and sulfur-containing detergent-type lubricant additive is a barium-containing neutralized reaction product of a phosphorus sulfide and an olefin polymer.

32. A method of inhibiting the corrosion of silver by a lubricant composition containing a sulfur-containing organic compound normally corrosive to silver, comprising incorporating in said lubricant composition a small amount, sufficient to inhibit said corrosion, of the reaction product of an aldehyde, a mercaptan selected from the class consisting of an aliphatic mercaptan and an aromatic mercaptan and 2,5-dimercapto-1,3,4-thiadiazole, said aldehyde, mercaptan and 2,5-dimercapto-1,3,4-thiadiazole being reacted in the molar ratio of from about 2:2:1, respectively, to about 10:2:9, respectively.

33. A composition comprising a major proportion of an oleaginous compound and from about 0.02% to about 10% of the reaction product of formaldehyde, tertiary dodecyl mercaptan, and 2,5-dimercapto-1,3,4-thiadiazole, said reactants being employed in the molar ratio of from about 2:2:1, respectively, to about 10:2:9 respectively.

34. A composition comprising a major proportion of an oleaginous compound and from about 0.02% to about 10% of the reaction product of ethyl hexaldehyde, tertiary octyl mercaptan, and 2,5-dimercapto-1,3,4-thiadiazole, said reactants being employed in the molar ratio of from about 2:2:1, respectively, to about 10:2:9, respectively.

35. A composition comprising a major proportion of an oleaginous compound and from about 0.02% to about 10% of the reaction product of benzaldehyde, tertiary octyl mercaptan, and 2,5-dimercapto-1,3,4-thiadiazole, said reactants being employed in the molar ratio of from about 2:2:1, respectively, to about 10:2:9, respectively.

36. A composition comprising a major proportion of an oleaginous compound and from about 0.02% to about 10% of the reaction product of furfural, tertiary octyl mercaptan, and 2,5-dimercapto-1,3,4-thiadiazole, said reactants being employed in the molar ratio of from about 2:2:1, respectively, to about 10:2:9, respectively.

37. A composition comprising a major proportion of an oleaginous compound and from about 0.02% to about 10% of the reaction product of heptaldehyde, thiophenol, and 2,5-dimercapto-1,3,4-thiadiazole, said reactants being employed in the molar ratio of from about 2:2:1, respectively, to about 10:2:9, respectively.

#### References Cited in the file of this patent

#### UNITED STATES PATENTS

|           |                 |               |
|-----------|-----------------|---------------|
| 2,414,257 | Evans et al.    | Jan. 14, 1947 |
| 2,515,318 | Schoene         | July 18, 1950 |
| 2,607,737 | Woodruff et al. | Aug. 19, 1952 |